

Aug. 15, 1972

W. H. BROWN

**3,684,563**

W. H. BROWN  
GALVANIZING CONTINUOUS ELEMENTS WITH PREVENTION  
OF CORROSION OF THE PAN

Filed Jan. 14, 1971

2 Sheets-Sheet 1



Inventor:

William H. Brown

By Hofgren, Wegner,  
Allen, Stellman, McCord *At this*

Aug. 15, 1972

W. H. BROWN

3,684,563

GALVANIZING CONTINUOUS ELEMENTS WITH PREVENTION  
OF CORROSION OF THE PAN

Filed Jan. 14, 1971

2 Sheets-Sheet 2



3,684,563  
**GALVANIZING CONTINUOUS ELEMENTS WITH  
PREVENTION OF CORROSION OF THE PAN**

William H. Brown, 6200 S. Adams St.,  
Bartonsville, Ill. 61607  
Filed Jan. 14, 1971, Ser. No. 106,442  
Int. Cl. C23c 1/02

U.S. CL. 117—114 A

9 Claims

## ABSTRACT OF THE DISCLOSURE

A method and apparatus for galvanizing steel wire including a corrodible electrically conductive pan containing a zinc bath through which the wire is moved lengthwise and in which the wire is brought to a temperature substantially above the inversion temperature with zinc within the bath, thereby creating current flow toward both the inlet and outlet ends of the bath within the wire. The method and apparatus involves the use of separate short circuits including a first short between the wire at the entry end of the bath and the wire at approximately its position of inversion temperature within the bath and a second short between the wires and the first and second intermediate sinkers, their position being at maximum wire potential in the bath beyond the inversion temperature position. Both of the short circuits are electrically insulated from the pan, thereby eliminating any corrosion-inducing current flow through the pan. The second short circuit also assures an even potential in the wire over a significant length of the bath to assure production of an even coating on the wire.

The bath includes an entry sinker bar which is electrically conductive and forms a portion of the first short circuit and two intermediate sinker bars which form a portion of the second short circuit. The first sinker bar is positioned at approximately the position of inversion temperature within the bath and the intermediate sinker bar are positioned at approximately the position of maximum potential above the inversion temperature position. The intermediate sinker bars are slightly lower in the bath than the other two bars to assure electrical contact of the wire therewith. Wires of any gauge can be galvanized in the same bath simply by regulating their immersion time in the bath to assure the desired coating weight.

## BACKGROUND OF THE INVENTION

### Field of the invention

This invention relates to the galvanizing of an elongated electrically conductive element by moving it lengthwise through a molten zinc bath. More particularly, the invention relates to a continuous method for galvanizing steel wire or steel strip by drawing it through a zinc bath in an electrically conductive corrodible pan and to the prevention of corrosion of the pan.

### Brief description of the prior art

It is a usual practice to galvanize a continuous element, such as a steel wire, by drawing the element from a source through a pan containing molten zinc to a take-up reel. A serious practical problem is the short life of the pan which tends to erode and fail, generally in the vicinity of the point of entry of the wire, usually after an average of only six to eight months. However, they have failed in thirty days.

I believe that pan erosion is caused by an electrochemical reaction resulting from a flow of electric current between the wire, the zinc and the pan. The current flow is established by thermoelectric potentials developed along the length of the wire as a result of temperature

differentials encountered in the galvanizing operation. Briefly, two types of potentials are present: (1) the potential resulting from the absolute temperature of the wire itself (the Thompson effect), and (2) the potential resulting from the temperature difference between the steel wire and the molten material in which it is immersed (the Seebok effect). The potentials due to the latter effect are of greater significance with respect to pan erosion.

10 In addition to pan erosion, current continuous galvanizing systems suffer other drawbacks which hamper production and decrease production rates. For example, the coatings vary over a wide range, requiring operating at reduced speeds to minimize the coatings below specifications. Also, the variations in coatings increase the zinc consumed per ton of wire, thus increasing the zinc cost by several dollars per ton of wire. Also, at time rejects due to low coating are high. In some cases, the coating thickness varies more than 75% on samples taken from a 20 single strand of wire.

## SUMMARY OF THE INVENTION

This invention provides a method and apparatus for galvanizing an elongated conductive metal element by moving the element lengthwise through a molten zinc bath contained in a corrodible container while blocking the flow of electric currents through the container, thereby inhibiting corrosion.

In a preferred form, the method and apparatus is 30 capable of galvanizing steel wire moved through the bath on a generally continuous basis. In the preferred bath container, the incoming sinker is located at approximately the position at which the wire reaches the inversion temperature with the zinc in the bath and the intermediate 35 sinkers are provided between the incoming sinker and the exit sinker at approximately the position where the wires reach maximum potential beyond the inversion temperature within the bath. In this form, two short-circuits are provided, one shorting the potential in the wires 40 between incoming sinker or position of inversion temperature with the wire prior to entry into the bath, and a second which shorts any potential differences in the wires between the intermediate sinkers. Both of the short-circuits are electrically insulated from direct contact with the bath container.

While this invention is susceptible of embodiment in many different forms, there is shown in the drawings and will be described herein in detail, a specific embodiment of the invention with the understanding that the invention 50 is not intended to be limited to such embodiment.

## BRIEF DESCRIPTION OF THE DRAWINGS

FIG. 1 is a plan view of a molten zinc bath useful in the method of the present invention;

55 FIG. 2 is a longitudinal section along line 2—2 of FIG. 1;

FIG. 3 is a section along line 3—3 of FIG. 2;

FIG. 4 is an enlarged section along line 4—4 of FIG. 1;

60 FIG. 5 is a plot of thermoelectric powers useful in understanding the present invention; and

FIG. 6 is a longitudinal section reduced from FIG. 2.

## DEVELOPMENT OF BACKGROUND MATERIAL AND STUDY OF THE PROBLEMS SOLVED BY 65 THE INVENTION

The present invention is the result of a new approach to solving the problems of pan erosion, dross formation and uneven coatings in galvanizing wire. Following my belief that pan erosion results from flow of electric currents through the bath and pan, I have studied the patterns of current flow through a galvanizing system. For

purposes of the following explanation of the background and the problem consider a molten zinc bath somewhat like that shown in FIG. 2 but in which the entry wire support bar 12 and exit drip bar or wiper 14 are mounted out of direct electrical contact with the pan 16, incoming sinker 18 and exit sinker 20 are secured by upstanding support arms in electrical contact with flange lip 22 of pan 16. And sinker bars 24 and 26 and contacts 28 and 30 are eliminated. Pan 16 contains a bath 32 of molten zinc at the normal process temperatures of about 460° C.

In a conventional galvanizing operation, the wire is drawn from a source such as a reel through an acid bath to clean the wire and then through a drying oven. From the drying oven the wire is drawn through the galvanizing bath, then in some cases through an annealing furnace at about 1000° F. and is then wound on a take-up reel. The method is continuous to the extent that an entire reel of wire is drawn through the complete galvanizing system and is taken up as galvanized wire on the take-up reel. The method continuously processes each reel of wire and during its travel through the system the wire passes across various supports and beneath sinkers in the various baths.

As shown in FIGS. 1 and 2, the wire 10 enters and passes through the galvanizing bath and is kept submerged in the bath by an incoming sinker 18 and an exit sinker 20. Plural wires may be processed at one time and the separate wires 10a, 10b, 10c, 10d, etc. can be recovered on separate take-up reels.

The steel wire elongated element 10 is a conductor and in a typical galvanizing apparatus, the wire is passed beneath the sinkers 18 and 20 which hold the wire submerged in the galvanizing bath. In prior systems, the sinkers were conductive elements mounted on the conductive flanges of the pan.

During the course of the galvanizing operation the temperature of the wire changes radically. Prior to entering the galvanizing bath the wire is at about ambient temperature and in the galvanizing bath the wire is heated to a temperature on the order of 460° C., i.e., the temperature of the molten zinc. The temperature variations along the length of the wire during heating within the galvanizing bath establish thermoelectric potentials in the wire. Referring to FIG. 2 of the drawing, if a potential reading is taken from a wire between point B at the incoming end of the zinc bath and point F at the exit of the bath, it is discovered that the potential not only varies over a wide range but at times the potential even reverses. I have found that when the exit end of the wire is positive in polarity, a potential in excess of two millivolts is often created and when the incoming end is positive, a potential in excess of one millivolt is often created. The potential varies between these limits, constantly changing or drifting up or down.

As an example of the variances in potential, I took potential readings from seven wires being run on a twenty-four wire frame over a twenty-four hour period, and the variance in these readings is given below:

| Wire No. | Potential variance<br>in millivolts |
|----------|-------------------------------------|
| 1        | -.3 to + .3                         |
| 4        | -.5 to + .3                         |
| 7        | -.3 to + .3                         |
| 10       | +.4 to +1.0                         |
| 13       | -.7 to +1.3                         |
| 16       | -.6 to 0                            |
| 19       | -.10 to +2.2                        |

The relative magnitudes of the Seebeck effect potentials are illustrated in FIG. 5. Where experimentally determined, thermoelectric powers for iron and zinc are plotted. The voltage which is developed as a result of a temperature difference between the junctions of the two dissimilar metals forming a potential depends on three factors: (1) the metals; (2) the difference of tempera-

ture between the junctions; and (3) the mean temperature of the two junctions. In a galvanizing process where a material is submerged in a hot bath of another material there are both a junction and a temperature differential over an extended length and the system is not susceptible of a simple quantitative analysis. However, a consideration of FIG. 5 will aid in a qualitative understanding of the problem. If, for example, there is a circuit of iron and zinc with one junction at 300° C. and the other junction at 400° C., the mean temperature is 350° C. and with references to FIG. 5, the thermoelectric potential difference is about 11 microvolts per degree. Since the temperature differential is 100° C., the generated voltage is about 1.1 of millivolts. Where the plots for iron and zinc cross at about 237° C., the polarity of the voltage developed in one portion of the system is the opposite of that in the other and the net voltage is the difference between the two. The point of intersection between the two is a neutral temperature or point of inversion for the two materials. If this temperature is the mean of the temperatures of the two junctions, no net voltage is generated.

Considering the inversion temperature of 237° C. in FIG. 5 as point "X" in the galvanizing bath of FIGS. 1 and 2, the potential "X-B" in the wire increases from point "X" to point "B", or cold end of the wire. Another potential "X-F" in the wire increases in the opposite direction from point "X" to point "F", or the high temperature end. Thus, in FIG. 2, current flows from point "X" toward both ends of the wire 10. Assuming that both the incoming sinker 18 and exit sinker 20 in the system of FIG. 2 are bolted in electrical contact to the flange 22 at the top of the pan 16, the following circuit is created: the wire 10 makes contact with the exit sinker 20 and through the exit sinker 20 to the pan flange 22, then through the pan sides and flange back to the ends of the incoming sinker 18 through the incoming sinker 18 to the wire 10 and then through the wire 10 into the exit sinker 20. This forms a complete circuit.

Returning to FIG. 5, it will be noted that there is a potential from the wire to the zinc coating when the temperature of the wire is equal to the temperature of the zinc bath, or 460° C. This potential difference is on the order of 20 microvolts. Additionally, when the sinkers have a zinc coating at the point of contact with the wire, the sinkers have an equal potential but the direction of the sinker potential is from the sinker to the wire. If the exit sinker 20 is coated at the point of contact with the coated wire 10, there are two opposing potentials at this junction.

At the incoming end of the bath, the incoming wire, being at about ambient temperature, lowers the temperature of a thin cover of zinc in contact with the wire for a short time. If it is assumed that the temperatures of the incoming wire and its coating have increased to the neutral inversion point, i.e., 237° C., by the time it reaches the incoming coated sinker 18, the potential between the wire and its zinc jacket is momentarily zero. But since the sinker 18 is coated at the point of contact of the wire, the potential of the sinker at bath temperature is from the sinker to the wire. The direction of this potential is the same as the "X-B" and "X-F" potentials so that the potential from the incoming sinker is added to the "X-B" and "X-F" potentials. If no current flows in the wire to reduce its potential, the potential from the incoming sinker 18 and the "X-F" potential will remain steady at a maximum value, resulting in a maximum uniform coating. However, the potential generally results in a current flow through the wire to the exit sinker 20 and through the circuit described above.

As indicated above, the "X-B" potential is developed in the incoming wire from a point near the incoming sinker to the point of initial contact of the wire with the molten zinc bath. The current from this potential flows in

the wire toward the point of contact with the zinc bath, then through the zinc bath to the incoming end of the pan or the sides of the pan near the incoming corners, then through the end of the pan to the sides of the pan and back toward the end of the incoming sinker 18. In the absence of any interference, the current would continue to flow through the pan sides and flanges to the ends of the incoming sinker 18 and through the sinker back to the wire, completing the circuit. However, the ends of the incoming sinker normally have a potential equal to or greater than the "X-B" potential because of the "X-F" potential described above. This forces the returning current resulting from the "X-B" potential to flow through the sides of the pan, near the ends of the incoming sinker and the zinc bath, back to the wire. If the resistance in the connection between the flange 22 of pan 16 and one or both ends of the incoming sinker 18 is high, some of the current resulting from the "X-F" potential is forced to flow through the side of the pan 16 near the ends of the incoming sinker 18 and the zinc bath 32 back to the wire 10. It is my belief that any current flowing through the sides of the pan to the bath reduces the life of the pan by causing corrosion or pitting.

The current flowing from the zinc-coated wire 10 to the exit sinker 20 deposits some of the zinc from the wire onto the exit sinker. As the zinc deposit builds up on the exit sinker, the opposing potential from the sinker increases, also the contact resistance, thereby reducing the current flow and increasing the "X-F" potential in the wire, also its coating. Thus, during the galvanizing operation the potential continuously varies and the thickness of coatings on the wire also normally varies.

As another consideration, it is often desirable to run a galvanizing unit using several different sizes of wires simultaneously, e.g., at 10a, 10b, etc. Also, at times, coating specifications may require running some of the wires at different speeds from other wires of different size. This creates poor conditions for forming uniform coatings because the resistance of different sizes of wire are not equal and the small wires come up to bath temperature and maximum potential in less time than the larger wires. Each of the wires being in contact with the incoming and exit sinkers and having maximum potentials at different positions in the bath causes circulating currents to flow between the different wires through the bath and sinkers. These circulating currents cause potential variations in the different size wires, resulting in variations in coating thickness. The range of coating variations is high in conventional galvanizing processes.

Variations in tension of the wires passing through the bath also cause coating variations. When the contact pressure between the wires and the sinkers increases, reducing the resistance of the contacts and increasing the current flow in the circuit, the "X-F" potential and the coating is reduced. Such variations in wire tension can result from variations in amounts of wire on the reels, the breaking effect of the reel breaks which are not always uniform, increased friction due to right angle turns in some of the wires before entering the galvanizing bath, and non-uniform take-up on the take-up reels, which often causes the reels to speed up or slow down, thereby changing the tension in the wires.

There are other factors contributing to variations in the potential and the current flow. Since the wire is under tension as it is being moved through the bath, a considerable amount of friction results between the wire and the sinkers and the friction wears through the zinc coating on the sinkers. As the sinker coating wears thin, the opposing potential from exit sinker 20 is reduced. This increases the current flow between the wire and the sinker and as a result of the current flow in the circuit, the potential of the source is reduced. The potential drop in the wire is equal to the current in amperes times the internal resistance of the potential source in ohms

and in a galvanizing bath the resistance of the potential source, i.e., the hot wire between the sinkers, is quite high so that a large drop in the "X-F" potential results with a relatively small current flow. Thus, as the current in the circuit increases the "X-F" potential drops and the current will increase until the potential drops to a value at which it cannot force any more current through the resistance of the circuit.

#### DESCRIPTION OF THE PREFERRED EMBODIMENTS

The form of the invention illustrated in the drawings is especially adapted to galvanizing steel wire which is drawn from a reel through the galvanizing process and coiled on a take-up reel. It is applicable not only to wire, but to strips and webs of other configurations. Further, it is not essential to the practice of the invention that the material to be galvanized be drawn from a reel or roll. For example, the wire can come directly from a wire-drawing die. Similarly, it is not necessary that the galvanized wire be wound on a take-up reel. It can be cut into short lengths and stacked, for example.

The embodiment shown in FIGS. 1-4 and 6 differs from a conventional galvanizing process. Accordingly, the incoming wire support bar 12 is electrically connected to the incoming sinker 18 by a pair of electric contact bars 28 secured to the ends of bar 12 and the ends of the incoming sinker 18. Also, sinkers 24 and 26 are provided at approximately the position of the maximum value of the "X-F" potential and the ends of sinkers 24 and 26 are secured to and in electrical contact with a second pair of electric contact bars 30 to which the ends of exit sinker 20 are also secured and on which the exit drip bar or wiper 14 is mounted so that bars 30 assure electric contact between sinkers 20 and 24 and 26 and wiper 14. The zinc bath and pan 16 is completely insulated from ground at all times during the operation of the apparatus.

The electric contact bars 28 and 30 are supported by and secured to the edge flange of pan 16 via electrically insulating mounting means 40. As best seen in FIG. 4, each insulating mounting means 40 includes a nut 42 welded to the top of flange 22. Insulating washers 44 and 46 and an intermediate insulating sleeve 48 are positioned in a base in contact bar 28 or 30 on top of the nut 42 as shown. A bolt 50 extends through the washers 44 and 46 and the sleeve 48 and is threaded into the nut 42. Washers 44 and 46, respectively, underlie and overlie the bar 28 or 30 and, with sleeve 48, completely insulate the bar 28 or 30 from the bolt 50, nut 42 and flange 22. Between the head of bolt 50 and the overlying insulating washer 46 there is provided a metal washer 52 which helps clamp washers 44 and 46 more securely against the faces of bar 28 or 30.

Each insulating mounting means 40 also includes a protective cover system for protecting the insulated connection. Accordingly, a cylindrical skirt 54 is provided welded to the bottom of bar 28 or 30 surrounding the nut 42 and spaced outwardly from the nut 42. The skirt 54 stops short of flange 22 to assure that no electrical contact is made between the protective cover and flange 22. Welded to the top of each bar 28 or 30 and around the bore is an upstanding cylindrical wall 56. Wall 56 surrounds but does not contact washer 52. The cylindrical wall 56 has external threads which receive a removable cap 58. The removable cap 58 permits easy access to the bolt 50 for tightening or loosening the mounting as desired.

In effect the contact bars 28 provide a low resistance short circuit across the "X-B" potential so that the potential is reduced to a very low value. This very low value results from the low resistance of a short piece of wire included in the circuit and the lower average temperature of the short piece of wire. The contact bar 12 being connected at each end to the bars 28 complete

a circuit from the incoming wires 10 to the contact bar, through the contact bar and the end connections to the ends of the incoming sinker 18 and through the incoming sinker 18 back to the wire 10, thus shorting the "X-B" potential. The shorting entry bar including the end connections and incoming sinker are all electrically insulated from pan 16 as a unit so that the "X-B" potential is reduced to a very low value and any possible current resulting from the "X-B" potential is prevented from flowing from the wire to the zinc bath then to the pan or from the pan into the zinc bath.

As described above, the ends of the exit sinker are mounted on bars 30 which are electrically insulated from the pan. This opens the circuit involving the "X-F" potential and prevents current from flowing through the sides of the pan, then through the zinc bath to the wire. Thus, the circuit described above with regard to "X-F" potential is broken and, since no current flows, the "X-F" potential remains at a higher average value. The higher average "X-F" potential in the wire results in a more uniform coating on the wire than when the exit sinker is electrically connected to the pan.

The sinkers 24 and 26 further assure the formation of uniform coating on the wires, even where wires of different size are simultaneously processed. As described above, sinkers 24 and 26 are insulated from the pan in the same manner as the other sinkers. Further, the sinkers 24 and 26 are spaced a distance from the incoming sinker 18 and are at a point along the bath where the "X-F" potentials in all of the wires have increased to the maximum value. For example, it requires approximately 3 1/4 seconds for a #9 wire to come up to bath temperature and maximum "X-F" potential and assuming this is the thickest wire to be processed, the intermediate sinkers 24 and 26 can be located at that point in the bath where the wire is at bath temperature when operating at maximum speed to obtain the required coating.

The angle of the wire making contact with the incoming sinker 18, also leaving exit sinker 20 is quite large resulting in increased contact pressure and low resistance connections. The angle of the wire making contact with sinker 24 is very small. This reduces the contact pressure and increases the contact resistance. The addition of sinker 26 with the ends of both sinkers 24 and 26 connected to conductors 30 results in the following. This forms two circuits in parallel reducing the contact resistance by 50%. Also, any variation in the wire potentials leaving sinker 24 are balanced by current circulating between the two sinkers in the end connecting conductors 30. This increases the stability of the potentials between sinkers 26 and 20, also the coatings.

It is believed that during galvanizing of wire using the present invention, the wire entering the molten zinc bath is covered with a thin layer of zinc and the zinc temperature at the wire is reduced by the cooler wire. As the wire travels further through the bath the wire temperature increases to bonding temperature and the zinc forms a bond on the wire. In the conventional process at times a large current caused by the "X-F" potential flows through the sides of the pan and the zinc to the wire at the beginning of the galvanizing bath. This current deposits a thick jacket of zinc on the wire. The heavy jacket of zinc deters the temperature rise in the wire so that the wire reaches the exit of the bath before its temperature is high enough to form a bond with the zinc, resulting in wire which must be scrapped. The present method eliminates the current flow to the wire at the incoming end of the bath, permitting the very thin cover of zinc on the wire to form and permitting the wire to heat to bonding temperature in less time. This assures good bonds at all times and leaves a greater percentage of immersion time for coating. The method thereby practically eliminates scrap, and it stabilizes the coating time and the coating weight.

A major advantage of the invention is that it increases the life of the galvanizing bath pan. Working with the

system has demonstrated that pan life may be increased from a few weeks or months to approximately that of the pans used when the hot dip method is applied. The potential differences do not occur with this method and the 5 pans often last from twelve to fifteen years. In one instance a pan was operated by a prior art process for about ten days and it was found that several pits developed in the bottom of the pan up to 1/4 inch in depth. For several years the pans on this frame had failed every five to 10 seven weeks, with an average of less than six weeks. After 15 then using the pan and operating under the present invention for a period of 4 weeks it was found that all of the pits had filled up with zinc. The pan was still in operation seven months later with no failure indicated. The extended life results in savings in material and down time.

Because of the uniform potential at maximum value 20 in the coating area of the present invention, the system can be operated at a faster rate with assurance that the minimum specified coating thickness is formed throughout 25 the length of the wire. This has resulted in a production increase of about 35%. If the heating capacity or the take-up frame limits the speed, shorter pans can be used, resulting in less cost. Operating at maximum speed increases the wire tension and improves the contact between 30 the wires and the sinkers. This improves the voltage control and reduces the coating variations. Increasing the operating speed reduces the immersion time and the coating weight. The optimum speed is the maximum speed below the required immersion time to assure the coating specifications.

Formation of dross is also reduced by about one-half 35 because of the insulating of the circuits and blocking flowage of current through the pan. Dross is believed to result from a current flowing from either the steel wire or 40 a steel pan into the zinc bath, causing disintegration of small particles of the steel. These particles of steel unite with the zinc to form the dross and the dross settles to the bottom of the pan and must be removed fairly frequently. The reduction of dross with the present invention results in saving of labor, down time and zinc which would otherwise be consumed in the dross.

I claim:

1. In a method of galvanizing an elongated conductive metal element by moving the element lengthwise through 45 a bath of molten zinc from an entry end to an exit end of the bath whereby the element is heated by the molten zinc within the bath beyond its inversion temperature with zinc so that current flows along the element toward both the entry and exit ends of the bath, the improvement comprising short-circuiting the entry end of said element with the portion of said element which is at about the inversion temperature.

2. The method of claim 1 wherein said bath is contained in an electrically conductive corrodible container 55 and said short-circuiting is by means electrically insulated from said container.

3. The method of claim 2 including the step of maintaining the portion of said element which has left the bath at the exit end out of electrical contact with the 60 container.

4. The method of claim 3 including the step of providing a stabilized potential in the element between the portion of the element at the exit end of the bath and the portion of the element within the bath which is at approximately maximum potential, above the inversion temperature and moving toward the exit end of the bath.

5. The method of claim 1 including the step of maintaining the portion of said element which has left the bath at the exit end out of electrical contact with the container.

6. The method of claim 5 including the step of providing more constant potential in the element between the portion of the element at the exit end of the bath and the portion of the element within the bath which is at ap-

proximately maximum potential, above the inversion temperature and moving toward the exit end of the bath, thereby providing a coating of more uniform thickness on the element.

7. The method of claim 1 adapted for operation in galvanizing elements of different cross-sectional areas and which are heated to inversion temperature by the bath at different rates, wherein a fixed inversion temperature position is provided for all elements moving through the bath in which said moving step comprises delivering the elements through the bath at a rate assuring that all of the elements are at inversion temperature at said position of inversion temperature. 5

8. The method of claim 1 wherein said element is steel wire of generally uniform diameter over its length which is moved as a generally continuous strand through the galvanizing bath. 15

9. The method of claim 8 wherein said element comprises a plurality of parallel strands of wire which are moved as separate generally continuous strands through the bath. 20

## References Cited

## UNITED STATES PATENTS

|            |         |            |             |
|------------|---------|------------|-------------|
| Re. 12,779 | 4/1908  | Goodson    | 117—93 X    |
| 1,053,664  | 2/1913  | Sommer     | 117—114 A   |
| 1,872,712  | 8/1932  | Fahrenwald | 118—429 X   |
| 1,890,463  | 12/1932 | Herman     | 117—114 A   |
| 2,063,721  | 12/1936 | Bradley    | 117—14 A UX |
| 2,286,194  | 6/1942  | Bradley    | 117—93 X    |
| 2,405,222  | 8/1946  | Mann       | 117—114 R X |
| 2,744,495  | 5/1956  | Boeghold   | 118—429     |

## FOREIGN PATENTS

|        |        |               |         |
|--------|--------|---------------|---------|
| 18,910 | 7/1907 | Great Britain | 117—128 |
|--------|--------|---------------|---------|

ALFRED L. LEAVITT, Primary Examiner

J. R. BATTEEN, Jr., Assistant Examiner

## U.S. CL. X.R.

117—128; 118—423